

Nov. 4, 1958

M. L. SUGARMAN, JR

2,859,352

ELECTRORADIOGRAPHY

Filed June 23, 1955

2 Sheets-Sheet 1

FORM X-RAY IMAGE OF  
OBJECT ON CHARGED  
PHOTOCONDUCTIVE  
COATING

DEVELOP ELECTROSTATIC  
IMAGE FORMED BY AND  
CORRESPONDING TO X-RAY  
IMAGE ON PHOTOCO-  
DUCTIVE COATING.

FIX DEVELOPED  
ELECTROSTATIC IMAGE  
TO PHOTOCODUCTIVE  
COATING

*Fig. 1*



*Fig. 2*

*Fig. 3A*



*Fig. 4*



*Fig. 3B*



*Fig. 3C*



*Fig. 5A*



*Fig. 5B*



*Fig. 6*

INVENTOR.  
MEYER L. SUGARMAN, Jr.

BY *J. L. Chittister*  
ATTORNEY

Nov. 4, 1958

M. L. SUGARMAN, JR.

2,859,352

ELECTRORADIOGRAPHY

Filed June 23, 1955

2 Sheets-Sheet 2



INVENTOR.  
MEYER L. SUGARMAN, JR.  
BY  
*J. L. Wittner*  
ATTORNEY

## 1

2,859,352

## ELECTRORADIOGRAPHY

Meyer L. Sugarman, Jr., Princeton, N. J., assignor to  
Radio Corporation of America, a corporation of Delaware

Application June 23, 1955, Serial No. 517,476

5 Claims. (Cl. 250—65)

This invention relates to improved methods and means for making radiographs (graphic recordings of X-ray images) electrophotographically. More particularly, the invention relates to improved electrophotographic methods and means for electroradiography employing a novel X-ray sensitive photoconductive material.

Previously radiographs or X-ray prints have normally been made on chemically developed film. X-ray processes using such film are expensive and time consuming. Furthermore, the methods using film require wet processes for developing and making prints. Often it is necessary to wait several hours before a usable print is obtained. Normally, in order to save time in obtaining usable results, the exposed negative is examined directly. The black-for-white reversed image involved is much more difficult to interpret than a direct positive image, such as that normally provided according to this invention.

It is therefore an object of this invention to provide improved methods and means for electroradiography.

A further object of the invention is to provide improved methods and means for producing usable radiographic prints directly upon an expendable X-ray sensitive material without the necessity of an intermediate dry or wet transfer step.

Another object of the invention is to provide improved methods and means for directly producing usable radiographic prints quickly and economically.

Still another object of the invention is to provide improved methods and means for directly producing a usable radiographic print on the object itself which is being inspected by X-rays.

Another object of the invention is to provide improved methods and means for directly producing usable radiographic prints within a few seconds after exposure without the necessity of an intermediate transfer step.

Yet another object of the invention is to provide improved methods and means for directly and continuously producing usable radiographic prints of a series of objects.

These and other objects and advantages of the invention are realized by a rapid dry process for directly making immediately usable radiographs. No transfer steps are necessary. In contrast to other dry electroradiograph systems using photoconductive selenium plates, for example, the X-ray sensitive material of the present invention does not require a transfer step, and does not require a special master plate which must be exposed over and over again, and cleaned between successive usages. In accordance with the invention, X-ray sensitive photoconductor-resin mixtures may be coated on paper, plastic, or metal sheets, for example, or directly upon the object to be examined. An example of such a material is finely divided ZnO dispersed in a silicone resin binder. An X-ray image of an object when formed on such a coating results in an electrostatic image corresponding to the X-ray image. The electrostatic image may be developed with a finely divided developer powder and fixed, as by

## 2

heating, or spraying with a quick-drying adhesive material.

The invention will be described in greater detail by reference to the accompanying drawing wherein:

5 Figure 1 is a diagram illustrating the steps of one method for carrying out the processes of the invention;

Figure 2 is a sectional, elevational view of one embodiment of apparatus in accordance with the invention for producing an X-ray image of an object on an X-ray sensitive photoconductive coating according to the invention;

Figure 3a is an elevational view of a completely assembled (potted) junction transistor whose internal structure is not visible to the unaided eye;

Figure 3b is a sectional, elevational view of apparatus for forming an X-ray image on an X-ray sensitive photoconductive coating of the internal structure of a transistor such as shown in Figure 3a;

Figure 3c represents a developed electroradiograph of the internal structure of the transistor shown in Figure 3a;

20 Figure 4 is a sectional, elevational view of another embodiment of the invention for producing an X-ray image on a photoconductive coating according to the invention;

Figure 5a is an elevational view of another embodiment of the invention wherein an X-ray image of the bone structure of the human arm is formed on an X-ray sensitive photoconductive coating directly upon the outer skin of the arm being X-rayed;

Figure 5b shows a developed electroradiographic print 30 of the bone structure of the human arm shown in Figure 5a;

Figure 6 is a partially schematic, elevational view of another embodiment of the invention for making radiographs of objects in a continuous process wherein the objects themselves are carried by an X-ray sensitive photoconductive-coated conveyor sheet;

Figure 7 is a partially schematic, elevational view of another embodiment of the invention for making radiographs in a continuous process on an X-ray sensitive 40 photoconductive-coated conveyor sheet; and

Figure 8 is a partially schematic, elevational view of still another embodiment of the invention for making radiographs in a continuous process directly upon the objects being inspected.

45 Similar reference characters are applied to similar elements throughout the drawing.

It is known that certain photoconductive materials may be employed to produce visible images by taking advantage of the electrical response of such materials to radiations such as visible light. Such materials may be charged electrostatically so as to hold a uniform electric charge. A charged layer of such a material, when exposed to light, will release its charge at whatever points the light impinges thereon by becoming more electrically 55 conductive at these points. Thus, a latent electrostatic charge pattern corresponding to the incident light image is formed on the coating. The intensity of the residual charge in different portions of the charge pattern is proportional to the intensity of the light received from different portions of the light image. This invisible latent electrostatic charge pattern may be rendered visible by developing with an electrically charged electrostatic powder which is attracted to and held by the charge pattern. This powder may be permanently fixed to the coating by 60 heating, solvent action, supplementary adhesives, or other techniques.

The photoconductive coating according to the invention comprises a finely divided photoconductive material dispersed in an electrically-insulating film-forming vehicle. It has been found that the materials according to the invention, in addition to being electrostatically responsive to light, are also sensitive to X-rays and may be em-

ployed to excellent advantage for almost instantaneously providing radiographs. According to the invention, the photoconductive material may be coated on paper sheets or rolls, metal or plastic films, glass plates or any other mechanically suitable surfaces to which the coating will adhere. Because of its cheapness, paper is preferred. As another important feature of the invention, the X-ray sensitive photoconductive material may be coated directly upon the object to be inspected radiographically.

The mixture used to produce the photoconductive coating may include a solvent or the mixture may be thermoplastic. The mixture may be coated by any convenient coating method, for example, by rolling on with a roller, by screening with a silk or metal screen, by brushing, by whirling, by spraying, or by stamping. After the mixture is coated, it is dried, for example by evaporation of the solvent, or by cooling if the mixture is thermoplastic. Where the coating is dried by evaporation, heat may be applied to accelerate the drying process. Similarly, the coating may be chilled where the mixture is thermoplastic and is applied hot.

When the photoconductive coating is produced on a backing of highly insulating material such as glass or high resistivity plastics, the backing may be treated so as to render its surface electrically conducting. This furnishes a plane immediately below the coating capable of being placed at ground or other desired potential in order to facilitate charging with a blanket electrostatic charge before exposure. This plane may be "floating" (isolated in potential) during all stages of image production other than charging. Preferably a double corona discharge is employed to provide ions of opposite charge on opposite sides of the coated insulating base so as to obviate the necessity of rendering a surface of the insulating base conductive.

#### X-RAY SENSITIVE PHOTOCODUCTIVE MATERIALS

Examples of suitable mixtures for producing an X-ray sensitive photoconductive coating are as follows:

*Example 1.*—A mixture of 80 grams of a 60% solution in xylene of silicone resin GE-SR-82, marketed by the General Electric Company, Silicone Products Division, Waterford, New York, 106 grams of toluene and 120 grams of photoconductive white zinc oxide is ball-milled for about three hours and then applied to the fixed form as described above.

*Example 2.*—A mixture comprising 100 grams of powdered photoconductive lead iodide, 100 milliliters of toluene and 60 milliliters of a 60% solution of a silicone resin (SR-82, source as above) in xylene is ball-milled until the lead iodide is thoroughly dispersed in the plastic-solvent mix and is coated as described above.

*Example 3.*—A mixture comprising 100 grams of finely ground photoconductive cadmium sulfide and 150 grams of a 35% polystyrene solution in toluene is thoroughly mixed for about 5 minutes in a high speed blender and coated as described above.

*Example 4.*—A mixture comprising 60 grams of a 35% solution of polyvinyl acetate resin in methanol, 40 grams of CP dry process white zinc oxide and 20 milliliters of acetone is ball-milled for about one hour and then coated as described above.

*Example 5.*—Equal parts by weight of CP photoconductive white zinc oxide and melted paraffin are intimately mixed and then the molten mixture applied as described above and then allowed to cool.

*Example 6.*—A mixture of three parts by weight of CP photoconductive white zinc oxide and one part by weight of carnauba wax are melted together and then coated as described above and then allowed to cool.

*Example 7.*—Three parts by weight of CP photoconductive white zinc oxide and one part by weight of carnauba wax are dissolved in toluene and then coated as described above.

*Example 8.*—Two parts by weight of CP photoconductive white zinc oxide and one part by weight of methyl cellulose are dispersed in a suitable solvent and then coated as described above.

*Example 9.*—Seven parts by weight of CP photoconductive white zinc oxide are dispersed in ten parts by weight of a 10% solution of a vinyl chloride, vinyl acetate copolymer resin in acetone. The mixture is thinned with acetone to the desired consistency and then coated as described above.

*Example 10.*—Ten grams of dry shellac are dissolved in 180 cc. of methanol and 20 cc. of acetone. 100 grams of this solution is mixed with 50 grams of CP photoconductive white zinc oxide and then coated as described above.

It was found that a mixture of zinc oxide and lead iodide had a greater sensitivity to X-rays than either material alone according to the examples above described. This mixture comprised about 10 grams of  $PbI_2$  to 90 grams of  $ZnO$  in the mixture.

#### FILM-FORMING VEHICLES

The electrically-insulating, film-forming vehicle is an essential part of the composition and may be chosen from any one of a number of substances. A preferred film-forming vehicle has a high dielectric constant and a high dielectric strength. These materials may be natural or synthetic resins or waxes. Examples of suitable resins are the vinyl resins, silicone resins, phenol-formaldehyde compositions, cellulose esters and cellulose ethers. Shellac is an example of a natural material. Examples of suitable waxes are paraffin, carnauba wax and beeswax. Inorganic binders such as sodium silicate may also be used. Mixtures including one or more vehicles may be used.

The photoconductor may be suspended in the vehicle in any of several ways. A simple way is to dissolve the film-forming vehicle in an organic solvent capable of effecting the solution and then dispersing the powdered photoconductor thereon. Alternatively the photoconductor may be dry blended by kneading with the film-forming vehicle heated to a sufficiently high temperature to be rendered plastic. In this case of waxes they may be melted and the photoconductor mixed with the melt.

The proportion of powdered photoconductor to film-forming vehicle in the final coating may vary over a wide range. The preferred ranges are 50 to 90% of photoconductor and 50 to 10% of film-forming vehicle. The optimum proportions will be based upon the nature of the photoconductor, the film-forming vehicle and the results desired.

The speed of response of the photoconductive coating is partially dependent upon the nature of the photoconductor material, the nature of the film-forming vehicle and the ratio by weight of the film-forming vehicle to that of the photoconductor. Since the speed of response depends on a balance of characteristics of these factors, almost any desired response may be obtained by a proper selection of materials and compositions.

A proper selection of materials and compositions will also designate how long an electrostatic image may be stored, since storage of the electrostatic image depends at least in part upon the resistivity of the coating. Generally the higher the resistivity of the coating the longer the storage time.

#### DEVELOPER MATERIALS AND APPLICATION

The developer powder may be applied in any of a number of ways such as by spraying, dusting, or brushing. For application by brushing a convenient brush comprises a mixture of magnetic carrier particles, for example, powdered iron and the developer powder. The mixture is secured in a magnetic field to form a developer brush. This method of development is more completely described by H. G. Greig in U. S. Patent application, Serial No. 344,123, filed March 23, 1953. A camel's hair-

or other brush comprised of bristles having suitable triboelectric properties to impart the desired charge to the powder may also be used.

A preferred carrier material for the developer mix in the magnetic developer system consists of "alcoholized iron," that is, iron particles free from grease and other impurities soluble in alcohol. These iron particles are preferably relatively small in size, being preferably in their largest dimension about .002" minimum to .008" maximum. Satisfactory results are also obtained using a carrier consisting of iron particles of a somewhat wider range of sizes up to about .001 to .020".

Other developing techniques are available and may be employed to advantage in any of the embodiments of the invention described. One method in particular may actually be preferred because of the sharply outlined images produced thereby. This technique is termed "cascade" development and is fully described by Robert C. McMaster in an article entitled "New Developments in Xeroradiography" published in the Journal of the Society for Nondestructive Testing Summer Number, 1951. In this technique the developing powders, consisting of a mixture of fine pigment particles and a coarse granular carrier material, are cascaded over the surface of the exposed plate in a rocking developing tray, for example. The images produced by this technique are high-contrast, sharp-line types rather than those of large areas of nearly constant density. Such images, of course, are highly desirable for some applications in radiography. This is particularly true where it is desired to accentuate small, but abrupt, changes in image density.

Another method which may be employed to develop the latent electrostatic images is placing the exposed photoconductor in an environment consisting of a cloud of electrically charged particles of powder. This technique is also described in the aforementioned article by McMaster.

A preferred developer powder may be prepared as follows: A mixture comprising 200 grams of 200 mesh Piccolastic resin 4358 (an elastic thermoplastic resin composed of polymers of styrene, substituted styrene and its homologs) marketed by the Pennsylvania Industrial Co., Clairton, Pa., 12 grams of Carbon Black 6, marketed by the Eimer and Amend Co., New York, N. Y., 12 grams of spirit Nigrosine S. S. B., marketed by the Allied Chemical and Dye Co., New York, N. Y., and 8 grams of Iosol Black, marketed by the Allied Chemical and Dye Co., New York, N. Y., are thoroughly mixed in a stainless steel beaker at about 200° C. The mixing and heating should be done in as short a time as possible. The melt is poured onto a brass tray and allowed to cool and harden. The hardened mix is then broken up and ball-milled for about 20 hours. The melted powder is screened through a 200 mesh screen and is then ready for use as a developer powder. This powder takes on a positive electrostatic charge when mixed with glass beads or iron powder. It therefore develops an electrostatic image composed of negative charges. 2-4 grams of the developer powder and 100 grams of the magnetic carrier material are blended together giving the completed developer mix. Other ratios may be used.

The developer powder may be chosen from a large class of materials. The developer powder is preferably electrically charged to aid in the development of the electrostatic latent image. The powder may be electrically charged because the powder (1) is electroscopic, or (2) has interacted with other particles with which it is triboelectrically active, or (3) has been charged from an electric source such as a corona discharge. Examples of other suitable developer powders are sulphur, natural and synthetic resins or mixtures thereof.

#### THE ELECTRORADIOGRAPHIC PROCESS

Referring to Figure 1, the steps of the method of the invention comprise the formation of an X-ray image of

an object to be examined on a blanket-charged photoconductive coating. This coating may be on a suitable backing such as paper or cellophane, metal, or glass, or upon the object itself. The X-ray image causes the photoconductive coating to become more conductive at the points receiving the radiation so that the charge at these points leaks off. Thus, the charges remaining (i. e., the "dark" areas not receiving X-rays) constitute a latent electrostatic image on the coating corresponding to the intensities in the X-ray image. This electrostatic image is then developed by applying a finely divided tone powder thereto. The powder deposits in densities proportional to the charge pattern, and may be fixed in place by a suitable method, such as by heating.

#### ELECTRORADIOGRAPHIC APPARATUS

Referring to Figure 2, an object 2 which is to be inspected is shown as being located between the X-ray apparatus 1 and the photoconductive plate 4. The X-ray apparatus is adapted to irradiate the object 2 with X-rays and to project an X-ray image thus formed upon the X-ray sensitive photoconductive coating 3 which has previously been charged with a uniform electrostatic charge. As is well known in radiography the precise distance of the object with respect to the X-ray source is not critical for focusing purposes if the X-ray source is a substantially point source as preferred in this and other embodiments of the invention. In general the distance of the object from the point source of X-rays and from the image plane determines only the enlargement of the image of the object from impingement of unabsorbed radiation from the X-ray source. Hence, the object 2 may be irradiated with X-rays whether spaced between the X-ray source 1 and the photoconductive coated plate 4 or placed directly on the plate as shown by dotted lines.

The sensitivity of the photoconductive coating may be appreciably improved by employing a metallic backing plate or intensifying screen just as in present radiography practice. The intensity of radiation is increased by such a plate due to the secondary emission of X-rays reflected back to the X-ray sensitive coating.

A latent electrostatic image is formed on the photoconductive coating 3 which corresponds to the X-ray image. After exposure the plate may then be removed and brushed, for example, with a finely divided developer as previously described to render the electrostatic image visible.

Referring to Figures 3a, 3b, and 3c, a typical use of the invention is illustrated. Figure 3a depicts the normally visual appearance of a potted junction transistor. Such devices are normally encased or potted in a small metallic cylinder or can or in a solid opaque block of a plastic such as a polymerized epoxy resin. The internal contents and structure thereof, of course, cannot be visually examined after the device is so potted. Usually such completed articles, if inoperative or defective, must be dis-assembled to determine the defect. According to the invention, a transistor such as shown in Figure 3a may be radiographed as shown in Figure 3b. In this embodiment the transistor 6 is shown as lying upon the charged X-ray sensitive photoconductive coating 3. After irradiation with X-rays and the development and fixing of the electrostatic image of the internal contents of the transistor formed thereby, a radiographic print is obtained as illustrated in Figure 3c. The total time involved in obtaining a completed print after exposure is only a few seconds. As shown in Figure 3c, the transistor 6 is inoperative due to a lateral crack in the germanium wafer. Thus, the defect causing inoperativeness is quickly and economically discovered. Alternatively, the radiographic print of the internal structure of the transistor can be made directly upon the external casing thereof by employing the technique described hereinafter in connection with Figure 4. Due to the low cost of the requisite materials according to the invention, and the easy and rapid processing in-

volved, it is feasible for the first time to make radiographic prints of each completed transistor or other articles of manufacture at the end of an assembly line production to detect possible defects such as thus described.

#### ELECTRORADIOGRAPHIC PRINTING ON X-RAYED OBJECTS

Figure 4 illustrates an important embodiment of the invention wherein the object 2 to be inspected by X-rays from the X-ray apparatus 1 is coated itself with the photoconductive material 3. Since the radiograph of the object 2 is to be formed actually on the object itself, the coating of photoconductive material is applied to the side of the object remote from the X-ray source and is then charged. Thus, the object actually is interposed between the X-ray source and the photoconductive coating. The X-ray image formed upon irradiation of the object in turn forms a latent electrostatic image upon the coating. This electrostatic image is rendered visible as before by applying a finely divided developer thereto. The developed image may be fixed in place as by heating, or may be removed, for example, by blowing off, or by brushing with a magnetic brush after dispersing the charge holding the powder image, for example, by exposure to light, and the coating re-used immediately or at a future time by re-charging, re-exposing with X-rays or visible light, and re-developing. Additional images may also be added by incidence of additional images of suitable spectral characteristics on non-image portions of the coated area.

By using the method of coating the object as illustrated in Figure 4, many advantages heretofore unobtainable with any previously known X-ray process may be realized. A radiograph of the contents of any opaque container may thus be printed upon the surface of the container showing not only the structure therein but also the shape, size, and position. This embodiment of the invention may be practiced to advantage in other applications such as in detecting flaws in metals which have been cast or machined. Here a radiograph showing the flaws may be printed directly upon the metal itself where the flaw occurs. As pointed out in connection with Figures 3a, 3b, and 3c the internal structure of devices such as a transistor showing size, position and defects, if any, can be printed directly upon the opaque casing in an assembly line technique.

Another important use of the embodiment wherein the X-ray sensitive photoconductive coating is applied directly to the object to be radiographed is in the field of medicine. Referring particularly to Figure 5a, a human arm is depicted which may have a bone fracture, for example. Heretofore prior to the setting of the bones it was necessary to X-ray the arm using chemically-developed film. After development of the film, which may consume several hours, the bone could properly be set by referring to the film. Furthermore, it is often desirable to have an indication on the limb itself representing the direction and location of the fracture. By prior methods this was accomplished by referring to the X-ray film in order to manually draw with an indelible pencil the approximate location and direction of the fracture. Finally, after the fractured arm or leg has been set, a cast is often placed thereon.

As shown in Figure 5a, the photoconductive coating may be applied directly onto the arm or to the outside of the cast on the side opposite the side to be exposed to X-rays. In order to charge the photoconductive coating 3 it is necessary to provide a conducting path to ground immediately below the photoconductive coating. The skin itself may be sufficiently conductive to provide this ground. Other additional grounding means may be easily and cheaply provided by first coating the skin surface with a thin film 7 of a colloidal graphite dispersion such as one of the "Dag" dispersions marketed by the Acheson Colloid Company, Port Huron, Michigan. Likewise silver platelet suspensions or other conducting

paints may be employed. The X-ray image thus formed on the photoconductive coating results in an electrostatic image which may be developed and fixed directly upon the arm itself or upon the cast. As shown in Figure 5b a radiograph 5 is thus obtained directly upon the member X-rayed showing not only the extent of the fracture but also its direction and location. Such a print is available within seconds after exposure to the X-rays. If it is desired to keep the area available for further radiographs, the fixing step may be omitted and after the fracture has been set the photoconductive coating with its visible image may be removed as by blowing off, by erasing with a magnetic brush after light exposure, or by washing with water or alcohol. To make later radiographs either on the arm or a cast it is only necessary to re-charge the photoconductive material and re-expose and develop.

#### ELECTRORADIOGRAPHIC CONTINUOUS PROCESSES

20 Referring now to Figure 6, a continuous process of electroradiography is shown for printing radiographs of a continuous series of objects 10 directly upon an X-ray sensitive photoconductive tape 12 which carries the objects. The paper which is coated with X-ray sensitive photoconductive material is supplied by the roll 14. This paper may comprise any grade of paper of reasonable strength. The coating comprises a finely divided photoconductive material dispersed in an electrically-insulating film-forming vehicle such as previously described.

25 30 The first operation is that of depositing a blanket electrostatic charge upon the photoconductive coating by means of the corona discharge apparatus 20 and a grounded metal plate 22. The paper passes between the corona discharge apparatus 20 and the grounded metal plate 22 which is necessary to aid in establishing the electric field necessary to produce a corona discharge. A grounded conductive roller may be used instead of the plate 22. The corona discharge apparatus may comprise three .003" diameter wires placed about 0.5" apart and about 0.5" from the surface to be charged.

35 The objects 10 to be electroradiographed are then placed on the charged photoconductive surface of the paper 12 and as the objects and the paper pass beneath the X-ray source 1 they are irradiated thereby. The X-ray image of the objects thus formed on the X-ray sensitive photoconductive coating in turn forms a latent electrostatic image corresponding thereto.

40 After exposure to the X-rays the objects may then be removed while the paper continues to travel to the developing station. The latent electrostatic images formed on the coating are brushed with a rotary magnetic brush 24. The magnetic brush may comprise a rotatable, circular magnet having attached thereto a mixture of finely divided magnetic carrier particles and finely divided developer particles. As the brush contacts the electrostatic images, the developer powder particles adhere thereto in a pattern corresponding to the electrostatic image. It is preferred to use the previously described developer mix which includes a thermoplastic developer powder.

45 60 After development the paper with its developed images thereon passes a heat source 26 which applies heat to the developed images, fusing the images and causing them to adhere to the photoconductive coating, thereby fixing the developed images to the paper 12. The heat source 26 may comprise a resistance heater or an infrared lamp. Thereafter the paper is wound upon a take-up reel 28.

65 70 A permanent radiographic record thus is obtained of each object coming off an assembly line production-type process, for example. In order to identify each object with its respective radiograph, X-ray opaque indicia may be placed on the objects so as to not obscure the structures thereof. An alternative indicia marking means takes advantage of the fact that the photoconductive ma-

terial is also light-sensitive. Thus the index information may be added by exposing the photoconductive coating at some convenient point to a visible light image using a suitable optical arrangement.

Another embodiment of the invention is shown in Figure 7 wherein a continuous series of objects 10 may be electroradiographed upon an X-ray sensitive photoconductive tape 12. In this embodiment the objects are not carried upon the X-ray sensitive tape itself but are transported by means of an X-ray transparent belt 30. Thus as the objects 10 are carried past the X-ray source 1, the X-ray images formed thereby are focused upon the X-ray sensitive paper which is being transported directly beneath the X-ray transparent belt 30. As before the X-ray sensitive paper 12 may be supplied already coated from the reel 14. Alternatively the paper may be fed uncoated past a coating-application trough 16 and coated thereby and then dried as it passes the heating source 18. Either an infrared lamp or an electrical resistance element may comprise the heating source 18. Other rapid drying means may be employed. Charging may be accomplished by means of a grounded metal roller 22 instead of but for the same purpose as the grounded plate described in connection with Figure 6. After the formation of the latent electrostatic image corresponding to the X-ray images, the paper is transported past the developer 24 and the fixer 26. This embodiment is especially advantageous where the weight of the objects to be electroradiographed is too great to be supported by the X-ray sensitive paper itself. In order to form sharp X-ray images of the objects upon the X-ray sensitive paper, the travel speed of both the conveyor belt 30 and the paper 12 must be substantially the same. Otherwise due to the movement of the objects 10 at a different rate with respect to the movement of the paper 12 during image formation blurring would occur. The synchronization of the belt conveyor 30 and the X-ray sensitive paper 12 may be accomplished by driving both the conveyor and the paper from the same motor 32 by like-diameter pulleys on the same motor shaft, and like-diameter pulleys on the paper take-up reel 28 and the conveyor belt driver 34. The X-ray transparent belt 30 may be made from any suitable X-ray transparent material having sufficient strength to support objects of given weights. An example of such a material is plasticised plastic-laminated fiberglass or cloth, or a thin aluminum or stainless steel belt. A sufficient intensity of X-rays to penetrate the belt completely should be employed.

In this embodiment a permanent radiographic print of each object is obtained. As explained before, the identification of a particular object with its image may be accomplished by placing X-ray opaque indicia upon the objects in some convenient location so as to not obscure any of the structure of the objects or by exposing to a visible light image of the indexing information.

Referring to Figure 8, a continuous process is shown for printing radiographs directly upon the objects to be examined by X-rays. The objects 10 are carried upon a continuous X-ray transparent conveyor 30 which may be made of any suitable X-ray transparent material sufficiently strong enough to support the objects. The conveyor 30 first carries the objects past a spray nozzle 16 which sprays the photoconductive coating completely over the upper surface of the objects. This coating comprises a finely divided photoconductive material dispersed in electrically-insulating film-forming vehicle such as previously described.

The photoconductive coated objects are then fed past an infrared lamp 18 or other heating means where the coating is dried. The next operation is that of depositing a blanket electrostatic charge upon the photoconductive coating on each object by means of the corona discharge apparatus 20 and 22 such as described previously. If the objects themselves are electrically conduct-

ing, a single corona discharge is sufficient. However, if the objects are relatively thin and flat but not electrically conductive, a second corona apparatus 22 furnishing a blanket charge of opposite electrical sign on the reverse side of the object may be aligned opposite the corona unit 20. The objects thus pass between the corona discharge apparatus 20 and the corona discharge apparatus 22 which is necessary to aid in establishing the electrical field necessary to produce a uniform surface charge.

10 The objects are thereafter passed over the X-ray source 1 and irradiated with X-rays therefrom. The X-ray image of the objects are thus formed on the X-ray sensitive coating on the objects themselves and these X-ray images in turn form latent electrostatic images corresponding thereto on the photoconductive coating on the objects.

15 The latent electrostatic images formed on the coatings on each object are then brushed with a rotary magnetic brush 24, or developed by other suitable means such as have been described. The magnetic brush (which may comprise a rotatable cylindrical magnet having attached thereto a mixture of finely divided magnetic carrier particles and finely divided developer particles) contacts the electrostatic images on the objects. The developer powder particles adhere to the images in a pattern corresponding thereto. Preferably a developer may be employed which includes a thermoplastic developer powder.

20 The last operation is performed as the conveyor 30 carries the objects with their developed images thereon past an infrared lamp 26 which fuses the images and causes them to adhere to the photoconductive coating on each object. The developed images are thereby permanently fixed to the objects themselves.

25 It has been found that the exposure time for the X-ray sensitive photoconductive materials such as zinc oxide or lead iodide is of the same order of magnitude as the exposure time of industrial X-ray film (type M, such as supplied by Eastman Kodak Co., Rochester, New York, for example).

30 40 It should be understood that the various charging techniques described are interchangeable and are primarily dependent upon the electrical characteristics of the material which is coated photoconductive. In general if the objects to be radiographed according to the invention are thin but not electrically conductive the double corona discharge apparatus described in connection with Figure 8 is to be preferred.

35 45 There thus has been described economically inexpensive methods and means for making radiographic prints either on a separate recording medium or upon an object being inspected radiographically. Many modifications of the invention may be made, as has been demonstrated, without departing from the scope of the invention. Because of the demonstrated versatility of the novel X-ray sensitive material according to the invention, many uses heretofore impossible or impractical may be realized. The instant specification has representatively illustrated the range of possible applications of the instant invention.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725

thereby formed on said coating produces a latent electrostatic image corresponding to said X-ray image, and developing said electrostatic image.

3. Electroradiograph apparatus comprising an X-ray transparent conveyor adapted to transport objects to be electroradiographed, means adjacent said conveyor for coating at least one side of each of said objects on said conveyor with a finely-divided photoconductive material dispersed in an electrically-insulating film-forming vehicle, means adjacent said conveyor for electrostatically charging said coating on said objects, X-ray means adjacent said conveyor for forming an X-ray image of each of said objects on said coating of each object as said objects are carried thereby, each of said X-ray images forming on said coating of each of said objects a latent electrostatic image corresponding to said X-ray image thereon, and means adjacent said conveyor for developing said electrostatic images as said conveyor passes thereby.

4. Electroradiograph apparatus comprising an X-ray transparent conveyor adapted to transport objects to be electroradiographed, means adjacent said conveyor for coating at least one side of each of said objects on said conveyor with a finely-divided photoconductive material, means adjacent said conveyor for electrostatically charg-

ing said coating on said objects, X-ray means adjacent said conveyor for forming an X-ray image of each of said objects on said coating of each object as said objects are carried thereby, each of said X-ray images forming on said coating of each of said objects a latent electrostatic image corresponding to said X-ray image thereon, means adjacent said conveyor for developing said electrostatic images with a finely-divided developer as said conveyor passes thereby, and means for fixing said developed images.

5. The method of claim 2 wherein said photoconductive material is zinc oxide.

References Cited in the file of this patent

UNITED STATES PATENTS

|           |                  |               |
|-----------|------------------|---------------|
| 2,221,776 | Carlson          | Nov. 19, 1940 |
| 2,666,144 | Schaffert et al. | Jan. 12, 1954 |
| 2,701,764 | Carlson          | Feb. 8, 1955  |
| 2,728,021 | Blanks           | Dec. 20, 1955 |

OTHER REFERENCES

"Large Area High-Current Photoconductive Cells Using Cadmium Sulfide Powder," Journal of the Optical Society of America, August 1955, vol. 45, No. 8, pages 647-650 especially p. 647.